

Jan. 31, 1933.

S. RUBEN

1,896,041

INSULATED WIRE

Filed May 2, 1931

*Fig. 1.*



*Samuel Ruben*

*Inventor*

*per* *Paul Robbins*

*Attorney*

## UNITED STATES PATENT OFFICE

SAMUEL RUBEN, OF NEW ROCHELLE, NEW YORK, ASSIGNOR TO VEGA MANUFACTURING CORPORATION, OF WILMINGTON, DELAWARE, A CORPORATION OF DELAWARE

## INSULATED WIRE

Application filed May 2, 1931. Serial No. 534,711.

This invention relates to an improved type of insulated wire.

An object of the invention is to produce a wire having a flexible refractory insulation.

A further object is the provision of a wire having a closely applied flexible insulating coating containing refractory inorganic material unaffected by high temperatures.

10 Another object is the provision of a wire having a refractory material applied and held on the wire by binders containing oil-resinous substances.

15 Another object is to provide a wire having a refractory insulation which is durable and waterproof.

Another object is to provide a refractory wire coating containing finely divided chromium oxide held upon the wire in flexible form.

20 Further objects will be apparent from the disclosure and drawing in which is shown an insulated wire made in accordance with this invention.

25 This application is a continuation in part of my application filed December 3, 1930, Serial Number 499,845. As stated in that application, I have found that in order to properly coat a wire with an insulating material having the desired characteristics it is desirable also to have (1) a flexible binder of the resinous type to give a proper bond at low temperature and (2) a further binder, which material is to be effective at high tem-

30 perature; this binder must be of the inorganic type such as boric acid or lead borate.

This second and most important binder serves two purposes; one, it binds the refractory and insulating material at high tem-

40 perature; two, it prevents scaling and undesirable surface oxidation. In the aforementioned application I described a coating comprising generally a refractory oxide, a gum or resinous binder and a borate or

45 other inorganic relatively high temperature binding agent. In the present case, the gum or resinous binder is specifically the oil enamel type. The oil-resinous binder, because of its high flexibility and water-

number of uses to the spirit varnish type of binder.

In the coating of this invention, the refractory oxide is preferably chromium sesqui-oxide although other materials have 55 been used with satisfaction such as aluminum oxide, magnesium oxide, beryllium oxide, titanium oxide, zirconium oxide, iron oxide, and combinations of these, chromium oxide being preferred over the other oxides 60 because of its high melting point and dielectric properties; also because under abnormal heat conditions it will not be broken down or detrimentally react with the oil-resinous binding materials used in the coating. Beryl or mica and even certain inert materials may also be added. The borate used is preferably boric acid although other borates may be used. The materials used should be ground to as fine a state as possible. 65 The organic binder or carrier is of the organic type, such as enamel.

The first step in the preparation of the coating is the production of a gum or resinous carrier of the enamel type. In a typical 75 enamel, I use 90 pounds of resin or gum, 10 gallons of tung oil, 5 gallons of linseed oil, 1 pound of lead acetate, 5 gallons of turpentine and 35 gallons of mineral thinner. The resin, tung oil and 3½ gallons of linseed oil 80 are heated to about 540° Fahrenheit. The mixture is then pulled from the fire, the lead acetate, the remaining gallon and half of linseed oil, the turpentine and the mineral thinner are added and the whole heated to 85 about 420° Fahrenheit.

A desirable coating is made by grinding materials in the following proportions: To 450 cc. of the prepared enamel I add 200 grams of chromium sesqui-oxide and 100 90 grams of boric acid, the mixture being milled until the various materials are thoroughly ground. The amounts given are not critical and the composition of the coating may be 95 varied by increasing or decreasing the respective amounts of the enamel or of the oxides, depending upon the flexibility or insulation desired; that is to say, when more oil enamel is used the flexibility is increased; and where 100

50 proofness due to the oil, is preferable in a

more oxide is used the refractoriness of the insulation is increased.

A continuous coating process is used in applying the insulation to the wire. The 5 wire passes through cups containing the insulating compound or mixture, being heated and baked in furnaces located between the cups. During the heating, the inorganic binder, the boric acid, melts and binds the refractory oxide crystals, a great part of the 10 organic materials being baked off.

Even though the wire, in use, is heated to a point where the organic binder, is disengaged, no harm results due to the presence of 15 the inorganic binder, boric acid. The use of this borate in the coating is also of assistance in dispensing with the necessity of a flux in soldering the wire, particularly when copper wire is coated.

20 The formula for making the enamel carrier or relatively low temperature binder may, of course, be varied. Practically all of the baking enamels will act as suitable carriers for the refractory oxide and the borate.

25 In the accompanying drawing, illustrative of the invention, the copper wire (1), has an insulating coating thereon consisting of a mixture (2) of an oil resinous varnish, finely divided chromium sesqui-oxide and boric acid which has been baked upon the wire.

I claim:

1. A wire having on its surface a closely adherent layer of flexible refractory insulation in which the refractory material consists 35 substantially of finely divided chromium oxide, held upon the wire by a baked oil-resinous enamel binder.

2. A wire having on its surface a closely adherent layer of a flexible refractory insulation consisting substantially of finely divided titanium oxide, held upon the wire by a baked oil-resinous enamel binder.

3. A wire having on its surface a closely adherent layer of a flexible refractory insulation consisting substantially of finely divided iron oxide, held upon the wire by a baked oil-resinous enamel binder.

4. An insulated wire having a coating of a finely divided insulating material held together with an enamel of the oil-resinous type and an inorganic binder capable of 50 withstanding high temperature.

5. A wire having on its surface a closely adherent layer of flexible refractory insulation 55 consisting substantially of the combination of non-fibrous inorganic insulating matter and an inorganic binding material, held upon the wire by an oil-resinous binder.

6. A wire having on its surface a closely adherent layer of flexible refractory insulation 60 consisting substantially of the combination of non-fibrous inorganic insulating matter and a boron compound, held upon the wire by an oil-resinous binder.

65 7. A wire having on its surface a closely

adherent layer of flexible refractory insulation consisting substantially of the combination of finely divided insulating oxide and a boron compound, held upon the wire by an oil-resinous binder.

70 8. A wire having on its surface a closely adherent layer of flexible refractory insulation consisting substantially of the combination of finely divided insulating oxide and boric acid, held upon the wire by an oil-resinous 75 binder.

80 9. A wire having on its surface a closely adherent flexible insulating layer consisting of a mixture of finely divided insulating oxide, an oil-resinous binding material and an inorganic binder compound effective at elevated temperatures.

85 10. A wire having a flexible insulating coating consisting of finely divided non-fibrous inorganic insulating material, a boron compound and an oil-resinous binding material.

90 11. A wire having a flexible insulating coating consisting of finely divided insulating oxide, a boron compound and an oil-resinous binding material.

95 12. A wire having a flexible insulating coating consisting of a plurality of baked on layers of a mixture of finely divided non-fibrous inorganic insulating material, an oil-resinous binder material and an inorganic binder compound, effective at elevated temperatures.

100 13. A wire having a flexible insulating coating consisting of a baked mixture of finely divided oxide, an oil-resinous binder material and an inorganic binder compound effective at elevated temperatures.

105 14. A wire having a flexible insulating coating consisting of a baked mixture of finely divided non-fibrous inorganic insulating material, an oil-resinous binder material and boric acid.

110 15. A wire having on its surface, a closely adherent flexible insulating layer consisting of a mixture of finely divided inorganic insulating material, a vegetable oil-resinous enamel and an inorganic binding material capable of withstanding high temperatures.

115 16. A wire having on its surface a closely adherent flexible insulating layer of a mixture of finely divided oxide, a vegetable oil-resinous enamel and an inorganic binding compound effective at high temperatures.

120 17. An insulated wire having a coating consisting substantially of finely divided oxide, a vegetable oil-resinous enamel and a boron compound.

125 18. An insulated wire having a coating containing finely divided chromium sesqui-oxide held together with an oil enamel binder and an inorganic binder effective at elevated temperatures.

130 19. An insulated wire having a coating containing finely divided chromium oxide

held together and upon the wire by an oil enamel binder and a second binder composed of a borate.

20. An insulated wire having a coating containing finely divided chromium sesquioxide held together and upon the wire by an oil enamel binder and a second binder of boric acid.

21. A wire having on its surface, a closely adherent flexible insulating layer consisting of a baked mixture of finely divided chromium oxide, an oil-resinous binding material and an inorganic binder compound effective at elevated temperatures.

22. A copper wire having on its surface a flexible insulating coating consisting of finely divided chromium oxide, an oil-resinous binding material and a boron compound.

23. A wire having a flexible insulating coating consisting substantially of finely divided titanium oxide, an oil-resinous binding material and an inorganic binder compound effective at elevated temperatures.

24. A wire having a flexible insulating coating consisting substantially of finely divided titanium oxide, an oil-resinous binding material and a boron compound.

25. A wire having a flexible insulating coating consisting substantially of finely divided iron oxide, an oil-resinous binding material and an inorganic binder compound effective at elevated temperatures.

26. A wire having a flexible insulating coating consisting substantially of finely divided iron oxide, an oil-resinous binding material and a boron compound.

In testimony whereof, I affix my signature.  
SAMUEL RUBEN.

40

45

50

55

60

65